

## UNITED STATES PATENT OFFICE.

WILHELM OERTEL, OF REMSCHEID-HASTEN, GERMANY, ASSIGNOR TO GLOCKEN-STAHLWERKE AKTIENGESELLSCHAFT VORM RICH LINDBERG, OF REMSCHEID-HASTEN, GERMANY.

## STEEL ALLOY.

No Drawing. Application filed July 31, 1924, Serial No. 729,370, and in Germany January 9, 1922.

Among steel alloys which are particularly resistant to disintegration by the atmosphere and by acids, alloys have been proposed, which besides iron contain chromium 5 as an effective component in quantities exceeding 8% and also carbon up to 1%. In general a chromium content of 12 to 20% and a carbon content up to 0.5% is used. Such alloys are generally termed stainless 10 steel.

It is known that this resistance to the action of acids and the atmosphere (referred to below as rust-proof quality) diminishes greatly when the carbon content exceeds 15 0.5%. This disadvantage has been overcome by the addition of quantities of nickel, for instance of 3 to 10%. One disadvantage of these alloys is that the presence of 20 large percentages of nickel entails the necessity of complicated methods of heat treatment for converting the steel, which shows of itself great hardness connected with considerable toughness, into a state, in which it can be machined. The high nickel content 25 also makes the steel less suitable for certain purposes, more particularly for tools with sharp cutting edges.

Neither the chromium steels nor the 30 chromium-nickel steels hitherto known are capable of withstanding the action of nitric acid with an addition of several per cent of alkali salt (e. g. chloride). They are also relatively easily attacked by hydrochloric acid and aqua regia. It is known 35 that chromium-iron alloys containing molybdenum are resistant to these agents, these cannot however be regarded as steel alloys but as iron alloys, as these contain carbon only as an impurity (say 0.05%). Such alloys 40 are sufficiently resistant to acids and acid mixtures with a content of alkali, more particularly alkaline chloride, of more than 5%. On the other hand as iron alloys they have the disadvantage that they cannot be 45 hardened.

Experiments have shown that it is possible to make a steel alloy which is capable 50 of being readily hardened, is proof against rust, has great strength, can be readily worked and is far more capable of resisting the action of acids and acid mixtures than the alloys hitherto known, if to a known

steel alloy with 8 to 25% Cr and 0.1 to 1.2% C is added molybdenum in quantities of from 0.2 to 6%. Manganese and silicon 55 may be present in the usual small quantities. This steel is even capable of resisting the action of boiling aqua regia for a considerable time.

The alloy according to the present invention with a content of chromium exceeding 15%, a carbon content up to 0.5% and a content of molybdenum up to 3% may be easily forged. When the content of carbon and molybdenum is greater, the forgeability 60 of the alloy decreases considerably. This disadvantage may be overcome by an addition of 0.5 to 2% Ni or 0.5 to 2% Co or by an addition of both elements up to 3% together. Nickel and cobalt are thus seen 65 to be (as is common in the art of alloys) largely equivalents for each other. The expression nickel-cobalt is intended to cover these two metals. By this addition the 70 rustproofness is not adversely affected, on the other hand the structure is rendered finer and the strength, more particularly the toughness, is greatly increased. The alloys containing above 0.2% C are capable 75 of being hardened and with about 0.5% C 80 are specially suitable for cutting tools. When annealed the alloy may be readily worked or stamped and may be rolled into thin plates or cold-drawn into wire. The annealing of the alloy presents no difficulties. 85

The recognition of the fact that the rust-proof quality of the alloy depends on the steel being very pure makes a thorough deoxidation necessary. It has been found to 90 be preferable to add vanadium or titanium up to 1% to the steel bath for obtaining thorough deoxidation. The two metals, being thus equivalents, to some extent, can be embraced within the expression "vanadium-titanium group."

Experiments have shown, that the alloy is also particularly suitable for making cast articles of all kinds, for instance vessels. In order still further to increase the fire-resistance of such articles, the content of molybdenum may be increased up to 10% 100 and the content of nickel or cobalt or the content of both these elements together up

to 15%. In this case as well the addition of vanadium or titanium to the steel bath in quantities up to 1% improves the purity of the steel and increases its resistance to the action of acids.

What I claim is:

1. A steel alloy, which is highly resistant to chemical action and is of great strength, consisting of iron, 8 to 25% Cr, 0,1 to 1,2% C, 0,2 to 6% Mo, and 0,5 to 3% of metal of the nickel-cobalt group for increasing the ductility of the alloy when hot.

2. A steel alloy which is highly resistant to chemical action and is of great strength,

consisting of iron, 8 to 25% Cr, 0,1 to 1,2% C, 0,2 to 6% Mo, and 0,5 to 3% of nickel and cobalt for increasing the ductility of the alloy when hot.

3. A steel alloy, which is highly resistant to chemical action and is of great strength, consisting of iron, 8 to 25% Cr, 0,1 to 1,2% C, 0,2 to 6% Mo, and 0,5 to 2% of Ni for increasing the ductility of the alloy when hot.

In testimony whereof I have signed my name to this specification.

DR. ING. WILHELM OERTEL.